

(No Model.)

H. PARTRICK.

SURGICAL SPLINT.

No. 336,740.

Patented Feb. 23, 1886.



Fig. 2.



WITNESSES.

*C. O. Perkins*  
*C. E. Ruggles*

INVENTOR,  
*Hawley Partrick*  
By  
*J. M. Wooster*  
Atty.

# UNITED STATES PATENT OFFICE.

HAWLEY PARTRICK, OF DANBURY, CONNECTICUT, ASSIGNOR OF ONE-HALF  
TO FRANK P. CLARK, OF SAME PLACE.

## SURGICAL SPLINT.

SPECIFICATION forming part of Letters Patent No. 336,740, dated February 23, 1886.

Application filed November 4, 1885. Serial No. 181,812. (No model.)

To all whom it may concern:

Be it known that I, HAWLEY PARTRICK, a citizen of the United States, residing at Danbury, in the county of Fairfield and State of Connecticut, have invented certain new and useful Improvements in Surgical Splints; and I do hereby declare the following to be a full, clear, and exact description of the invention, such as will enable others skilled in the art to 10 which it appertains to make and use the same.

My invention relates to that class of surgical splints which in use are softened, and while in a plastic condition are applied to that portion of the person which they are intended to 15 support, and which will quickly set and harden in any form which they may be caused to assume; and the object of my invention is to produce a splint of this general class which may be readily and thoroughly softened with 20 out dipping into boiling water, but which may be placed in boiling water without injuring it in the slightest, which will set and harden very quickly, and which, after hardening, will be stiffer and harder than any splints of this class 25 now in use.

It has heretofore been a serious objection to surgical splints as placed upon the market that they required to be dipped in boiling water to soften them. This is an unpleasant operation, 30 and is frequently exceedingly painful both to the operator and to the person operated upon.

In order to overcome the above-stated objections and to produce a surgical splint which shall be economical in cost and thoroughly acceptable both to the surgical profession and to wearers, I have devised the novel splint and method of making the same, of which the following description, in connection with the accompanying drawings, is a 40 specification.

Figure 1 is a perspective, and Fig. 2 is a plan, view of a splint of this class formed to the shape of a human arm, and adapted to hold the ulna and radius at a right angle to the humerus, it being understood, however, 45 that the special portion of the body to which the splint may be formed has nothing whatever to do with my invention.

In manufacturing my improved splint I use 50 a good quality of fur instead of wool, or wool

and fur, or wool and hair, as has heretofore been the practice.

My improved splints are stiffened by a special compound, which I have found after long-continued experiments to be especially adapted 55 for this purpose. This compound consists, preferably, of eighty parts shellac, sixty parts resin, and thirty parts gum-thus, dissolved, preferably, in ammonia-water, although other solvents—as, for example, a saturated solution 60 of borax (baborate of soda)—may be used, if preferred.

The method of manufacturing is as follows: The felt is made by blowing the fur upon a cone in precisely the same manner that hat-bodies are formed. It is then shrunk in the usual manner and dried, after which it is stiffened by dipping in the special stiffening compound described and wringing out, after which it is dried again. The next step in the process 70 is to put the pieces of felt, after they have been stiffened and dried, in a hot-steam box for about three-quarters of an hour, the effect of which is to drive the stiffening from the surface into the felt, leaving the surface perfectly 75 soft and smooth. The pieces of felt are then cut up into strips of suitable shape and size and are stretched over forms. The strips are of course made plastic for stretching by heating them, and are stretched over the forms 80 while hot, using either the hands or a tool for the purpose of forming them.

It will of course be understood that the proportions stated of the stiffening compound may be varied within reasonable limits without departing from the spirit of my invention. I have merely given certain proportions which I have found desirable in use.

Having thus described my invention, I claim—

1. As a new manufacture, a surgical felt splint adapted to be softened by heat alone and to set and harden quickly, said splint being made of fur and stiffened by a solution of shellac, resin, and gum-thus.

2. As a new manufacture, a surgical splint made of fur and stiffened by a compound of shellac, resin, and gum-thus, in substantially the proportions stated, dissolved in ammonia-water.

3. The method of making surgical splints, which consists in forming, shrinking, and drying the felt in the usual manner, then stiffening by dipping in a solution of shellac, resin, and gum, thus, wringing out and drying again, then subjecting to the action of steam for substantially the time stated, and finally cutting into strips for use.

4. The method of making surgical splints, which consists in forming and shrinking the felt in the usual manner, then stiffening with a compound of shellac, resin, and gum, thus, in substantially the proportions stated, in solution, then subjecting to the action of steam, then cutting to strips of desired shape and size, and finally forming to the desired shape while in a plastic condition.

5. The improvement in the art of making splints, which consists in forming, shrinking, and drying the felt, then dipping in a compound of shellac, resin, and gum, thus, in substantially the proportions stated, dissolved in ammonia-water, then drying again, then subjecting to the action of steam to soften the outside, and finally cutting into strips for use.

In testimony whereof I affix my signature in presence of two witnesses.

HAWLEY PARTRICK.

Witnesses:

A. M. WOOSTER,

C. E. RUGGLES.